

Patented June 11, 1929.

1,716,943

# UNITED STATES PATENT OFFICE.

ROBERT S. ARCHER AND WILLIAM L. FINK, OF CLEVELAND, OHIO, ASSIGNEES TO ALUMINUM COMPANY OF AMERICA, OF PITTSBURGH, PENNSYLVANIA, A CORPORATION OF PENNSYLVANIA.

## ALUMINUM-BERYLLIUM ALLOY AND METHOD OF TREATMENT.

No Drawing.

Application filed November 22, 1926. Serial No. 150,141.

The invention relates to aluminum base alloys containing beryllium, one object being to provide a method of heat-treating such alloys to improve their physical properties, 5 and another to provide improved aluminum-beryllium alloys which have substantial advantages without as well as with heat-treatment.

Because of its low density, beryllium is a 10 desirable alloying element for many purposes for which light aluminum base alloys are used, but because of its present high cost, beryllium cannot be used in large quantities as an alloying constituent in competition 15 with less expensive alloying constituents. We have discovered, however, that by alloying relatively small quantities of beryllium with aluminum there result inexpensive light aluminum base alloys, which, when heat-treated in a particular manner discovered by 20 us, possess materially higher physical properties than previously known similar aluminum-beryllium alloys. As to this heat-treatment, we have discovered that aluminum-beryllium alloys, particularly when 25 made from quite pure metals, possess a marked increase in hardness and tensile strength when heated for a substantial period of time at a temperature slightly below the aluminum-beryllium eutectic temperature and then quenched in water or another suitable quenching medium. We have also discovered that aluminum-beryllium alloys 30 when thus heat-treated, age harden, both naturally at room temperatures, and artificially at temperatures not higher than about 200° C.

In the practice of the feature of our invention having to do with a method of heat-treating aluminum base alloys containing beryllium, such an alloy is heated to a temperature slightly below the melting point of the most fusible constituent of the alloy, which may be that of the aluminum-beryllium eutectic, and is maintained at such temperature 45 for a substantial period of time, the alloy being then quenched at, or substantially at, the temperature to which it was heated. We have found that the temperature to which the 50 alloy is heated and at which it is maintained may vary from about 550° C. to slightly below 645° C., which latter is about the alu-

minum-beryllium eutectic temperature. The period of time during which the alloy is maintained at an elevated temperature varies 55 with its size and with the heating temperature and the beryllium content of the alloy. The time of heat-treatment will also vary according as the alloy is in the cast condition or has been mechanically deformed. However, this 60 may be readily determined by practice and from the illustrative examples of the invention presently to be described.

After an aluminum-beryllium alloy has been so heated and quenched, it is age hardened either naturally at room temperature or artificially at an elevated temperature not higher than about 200° C. We have found that an aluminum-beryllium alloy, for example a binary alloy in the form of a casting, 70 age hardens naturally at room temperature quite rapidly, and that this hardening is often substantially complete after one or two days. However, it is sometimes advantageous to effect the age hardening artificially at elevated 75 temperatures.

As has been stated, the effect of this heat-treatment is to substantially increase the hardness and tensile strength of the alloy. As cast, the alloy may contain undissolved 80 beryllium, which, upon being heated in the manner explained, tends to dissolve and form a solid solution up to the solubility limit at the temperature to which it is heated. When the alloy is quenched from this temperature 85 the solid solution is retained at room temperature, and, upon aging, the excess constituent which was dissolved at the higher temperature tends to precipitate in the form of very small particles which harden and stiffen 90 the matrix, thereby increasing the strength and hardness of the alloy.

Aluminum-beryllium alloys such as herein contemplated may be variously manufactured. For example, an alloy of low beryllium content may be prepared by stirring metallic beryllium, which melts at about 1280° C. in molten aluminum at about 1100° C. until the beryllium is dissolved. The use of small amounts of a flux such as barium chloride 95 facilitates introduction of the beryllium. By using higher temperatures, rich aluminum-beryllium alloys containing 10, 25 or 50 per cent or more of beryllium may be prepared 100

in this way for use in the subsequent preparation of aluminum-beryllium alloys having lower beryllium content, or for use themselves without subsequent alloying.

5 The invention will now be further explained with reference to specific examples with the understanding, however, that the examples are given by way of illustrations and not as limitations of the invention.

10 In the following table there are given in the first column the beryllium content of a number of aluminum-beryllium alloys, specimens of which were prepared by casting the alloys in iron molds to give chill cast slabs 15 about one-fourth of an inch thick. The Brinell hardness values of these alloys as cast were determined by using a 10 millimeter ball under a load of 500 kilograms, and are given in the second column of the table. The several 20 specimens were then all heated for 24 hours at a temperature of 631° C. and then quenched in water, after which their Brinell hardness values given in the third column of the table were determined in the manner just explained. 25 Thereafter the specimens were all permitted to age naturally for two days at room temperature, and their Brinell hardness values given in the last column of the table were then determined.

|    | Beryllium per cent | Hardness as cast | Hardness quenched | Hardness when aged 2 days at room temperature |
|----|--------------------|------------------|-------------------|-----------------------------------------------|
| 30 | 0.013              | 16.8             | 15.7              | 16.9                                          |
| 35 | 0.025              | 17.2             | 17.2              | 24.3                                          |
|    | 0.075              | 19.4             | 22.7              | 36.8                                          |
| 40 | 0.21               | 21.2             | 23.8              | 37.0                                          |
|    | 0.40               | 22.8             | 24.1              | 39.1                                          |
|    | 0.75               | 25.9             | 27.3              | 42.9                                          |

45 This table shows that the Brinell hardness values of the specimen containing .013% beryllium do not vary materially with heat-treatment, the hardness value of the specimen when quenched and aged being substantially the same as when cast. However, the specimen having a beryllium content of .025% when quenched and aged had a Brinell hardness materially higher than as cast or as 50 quenched, and this is likewise true of the several specimens having beryllium contents greater than .025%. From this it appears that aluminum base alloys containing not less than about .025% beryllium are capable of 55 having their hardness and strength substantially increased by heat-treating them according to this invention.

60 Several tests were made to determine the effect of heating the alloys at temperatures above and below that used in heating the specimens given in the above table. A specimen of an alloy containing .075% beryllium after being heated for 18 hours at 637° C., 65 quenched in water and aged three days at

room temperature was found to have a Brinell hardness of 24 immediately after quenching, and of 45 after aging. Other specimens of the same alloy after being heated for 18 hours at 600° C. and quenched in water were 70 found to have an average Brinell hardness value of 25 as quenched, and of 40.2 after aging at room temperature, showing a decrease in Brinell hardness as compared to the sample which was heated at 637° C. but nevertheless showing a substantial increase in hardness as compared to that as quenched. 75

Still further samples of the same aluminum-beryllium alloy after being heated for 18 hours at 600° C. and quenched in water 80 were found to have a Brinell hardness of 25.4. One sample was artificially aged for three hours at 150° C. and found to then have a Brinell hardness of 34.4. Another sample showed a Brinell hardness of only 27.1 after 85 aging 50 hours at room temperature, showing that the age hardening is more rapid at elevated than at room temperatures.

Similar tests have been made of various other alloys containing different percentages 90 of beryllium with results of the same general order as typified by the examples just explained. As showing that the invention is applicable to aluminum-beryllium alloys containing much larger percentages of beryllium, an alloy containing 23% beryllium after being heated for 18 hours at 638° C. and quenched in water was found to have a Brinell hardness of 30, and after being aged for 100 two days at room temperature the Brinell hardness was found to be 38.

The invention is applicable not only to chill castings made of aluminum-beryllium alloys, but also to sand castings, as shown by the following example. Samples of sand cast aluminum-beryllium alloys containing .5% beryllium showed in the cast condition an average tensile strength of about 12,000 pounds per square inch and a Brinell hardness of 21. After aging 11 days at room temperature the 110 samples showed no appreciable change in strength or hardness. Other samples of the same alloy after being heated for 30 hours at 632° C. and quenched in water had a tensile strength of 13,000 pounds per square inch 115 and a Brinell hardness of 23. These heat-treated samples were then permitted to age naturally at room temperature for 11 days, when it was found that their average tensile strength was 17,000 pounds per square inch 120 and their Brinell hardness 36.

The samples thus far given have been of cast aluminum-beryllium alloys, but the invention contemplates wrought, rolled or otherwise worked alloys. As illustrative of this, an alloy containing 0.075% beryllium was forged hot to a bar about five-eighths of an inch square, and after annealing was found to have a Brinell hardness of 16.4. 125 The sample was then heated for 20 hours at 130

631° C., quenched in cold water, and then permitted to age naturally at room temperature. After so aging for 16 hours its Brinell hardness was 31, and at the end of 72 hours it 5 was 34.

This same heat treatment process can be applied with advantage to sheet rolled from the aluminum-beryllium alloys. Such alloys were made up to contain varying amounts 10 of beryllium, ranging from 0.0125 to 23.0 per cent, using aluminum of about 99.9% purity. We found that sheet 0.064 inches thick can be rolled readily from small ingots of these alloys. Two samples illustrative of the beneficial effect of our heat treatment upon sheet material 0.064 inches thick are given in the following table.

| Beryllium per cent | Annealed state |                  |            | Heat-treated state |                  |            |
|--------------------|----------------|------------------|------------|--------------------|------------------|------------|
|                    | Yield point    | Tensile strength | Elongation | Yield point        | Tensile strength | Elongation |
| 0.075              | 2800           | 9255             | 48.0       | 12050              | 15395            | 19.5       |
| 23.0               | 16380          | 26460            | 12.5       | 24250              | 31080            | 11.0       |

In this table the sheet in its annealed state had been annealed at 300° C., and in its heat-treated state it had been heated for one and one-half hours at 625° C., quenched in cold water, and aged several weeks at room temperature. The yield points and tensile strengths are given in pounds per square inch, and the elongations in per cents in two inches.

Heat-treatment of aluminum-beryllium alloy sheet also serves to increase the corrosion resistance as determined by the usual salt spray method. In applying this test the changes in elongation are usually considered 35 to constitute a more sensitive criterion of the corrosion effect than the changes in tensile strength. Samples of sheet rolled from the aluminum-beryllium alloy were exposed 40 to salt spray for 1300 hours, with the following results in elongation which is given in per cent in two inches.

| Beryllium per cent | Condition                          | Elongation before corrosion | Elongation after corrosion |
|--------------------|------------------------------------|-----------------------------|----------------------------|
| 0.075              | Annealed                           | 48.0                        | 43.1                       |
| 0.075              | Heat treated 625° C., and quenched | 19.5                        | 21.4                       |
| 23.0               | As rolled                          | 4.0                         | 1.63                       |
| 23.0               | Heat treated 625° C., and quenched | 11.0                        | 12.3                       |

These figures show that heat-treated sheet specimens are much less affected by the salt spray than sheets which are in the as rolled or annealed condition.

As previously indicated, a further feature of our invention has to do with the provision of ternary or more complex aluminum alloys containing beryllium. We have found very useful and beneficial effects are produced by 60 the addition of beryllium to aluminum base

alloys containing silicon, copper, magnesium, magnesium and silicon, magnesium and copper, and magnesium, copper and silicon. Depending upon the particular alloy in question, the effect of the addition of beryllium to these 70 alloys may, for example, be to confer age hardening characteristics where they did not exist before, to increase the age hardening characteristics already inherent in the alloy, and to increase the total hardness of the 75 alloy.

As shown by the following example, beryllium confers age-hardening properties upon chill cast aluminum-copper alloys. Such an alloy containing 4% copper and no beryllium 80 after being chill cast showed no appreciable increase in hardness after standing several days at room temperature. However, when .05% of beryllium was added to an aluminum base alloy containing 4% copper and the alloy chill cast, the Brinell hardness increased from 46 immediately after casting to 69 after the sample was aged naturally for five days at room temperature. Similarly, the Brinell hardness of an aluminum alloy containing 90 3% copper and 0.05% beryllium increased from 48 as cast to 64 after aging eight days at room temperature. After heating samples of the last mentioned aluminum-copper-beryllium alloy for eight hours at 589° C. 95 and quenching in water, it was found that the Brinell hardness as quenched was 58, and after aging two days at room temperature it was found that the hardness had risen to 87. Results of the same order were obtained by 100 varying the beryllium as well as the copper content of other aluminum base alloys containing these constituents.

Heat-treated pure aluminum-copper alloys show distinct hardening at room temperature. For example, an aluminum-copper alloy containing 4% copper was heat-treated at 105 550° C. and quenched. The hardness of the as quenched specimen was 63. After aging twenty-five days at room temperature, the 110 hardness had increased to 79. The addition of beryllium to such an alloy causes an increase in this effect. The addition of 0.05% beryllium to the foregoing alloy caused the hardness to increase from 65 immediately 115 after quenching from 550° C. to 99 after aging twenty-five days at room temperature.

It is shown in the following example that the addition of beryllium to aluminum-copper alloys has the further advantage of reducing the liability of the alloy "burning" during its forging or heat-treatment. The heating curve showing the increase in temperature per unit of time of an aluminum-copper alloy containing 6% copper normally 120 shows an arrest when the alloy reaches a temperature of about 548° C., this being due to the fusion of the aluminum-CuAl<sub>2</sub> eutectic at this temperature. When .81% of beryllium was added to an aluminum-copper alloy con- 130

taining 6% copper and the resulting alloy heated, it was found that the first arrest in the heating curve was at 564° C. and that forgings of this alloy heat-treated for two and one-half hours at 554° C. showed no signs of "burning." This indicates that the copper and beryllium had probably combined in some way, because otherwise any free CuAl<sub>2</sub> present in the alloy would have 10 melted at or below the aluminum-CuAl<sub>2</sub> eutectic temperature of about 548° C.

We have found that in some cases heat treating periods much shorter than some of those used in the preceding examples produce 15 equally beneficial results. As illustrative of this, samples of a forged aluminum-copper-beryllium alloy containing 6% copper and .81% beryllium were heat-treated for two and one-half hours at 554° C. and 20 quenched in water. As determined by using a 1000 kilogram load, the Brinell hardness of this alloy as quenched was 69, and after aging naturally at room temperature for twenty-four hours it had risen to 98. At the end of 25 forty-eight hours the Brinell hardness was 99, and at the end of twelve days it was 101. The average tensile strength of forged samples of this alloy after aging twelve days was found to be about 52,000 pounds per square 30 inch, and the elongation to be 25% in two inches.

As to the effects of beryllium on aluminum base alloys containing additional alloying constituents other than copper, we have 35 found by a number of tests that the addition of silicon to aluminum beryllium alloys results in an increase of their final hardness after quenching. An aluminum base alloy containing .1% beryllium, .5% magnesium 40 and 1% silicon was found to have a Brinell hardness of 42 as cast and of 54 after aging for one week at room temperatures, the latter being materially higher than that of a similar alloy not containing beryllium. 45 After being heated for eighteen hours at 550° C., quenched in water and aged for one week at room temperature the Brinell hardness of the aluminum-beryllium-magnesium-silicon alloy just described was found 50 to be 74. An alloy of the same composition plus 4% copper showed as cast a Brinell hardness of 70, and after aging at room temperature for one week it showed a Brinell hardness of 84. Samples of this alloy, after being 55 heated for fifty hours at 500° C. and quenched in water, showed as quenched a Brinell hardness of 57, and after aging at room temperature for one week a Brinell hardness of 97.

From the foregoing it clearly appears that 60 certain aluminum base alloys containing beryllium, whether they are binary, ternary or more complex alloys, have their physical properties substantially increased by heating them for a substantial period at a temperature slightly below the melting point of the

aluminum-beryllium eutectic, or in the case of the ternary and more complex alloys to a temperature slightly below the melting point of the most fusible constituent of the alloys, and then quenching them. In general, regardless of the temperature at which an aluminum-beryllium alloy may be treated, it is necessary to heat the alloy only long enough to cause substantial solution of the undissolved beryllium constituent. It is also 75 evident from the foregoing examples of aluminum base ternary and more complex alloys containing beryllium that they possess substantial advantages whether or not they are heat-treated according to the method here 80 provided. When it is desired to age the heat-treated alloys at elevated temperatures, it is possible to quench them from the heat-treating temperature in boiling water or other suitable medium at the desired temperature 85 and to maintain them at this temperature for an appropriate length of time.

Throughout this specification, and in the appended claims, the expression "aluminum base alloy" is used to describe an alloy in 90 which aluminum is the predominant constituent regardless of whether the alloy is binary, ternary, or of a more complex order.

No claim is made in this application to the improved alloys which we have disclosed, 95 such alloys being claimed in a divisional application.

According to the provisions of the patent statutes, we have explained the principle and mode of operation of our invention and have 100 described numerous specific examples of the manner in which it may be practiced. However, we desire to have it understood that, within the scope of the appended claims, the invention may be practiced otherwise 105 than as explained with reference to the examples given, and in alloys having compositions differing from those particularly described.

We claim as our invention:

1. The method of treating an aluminum base alloy containing beryllium, which comprises heating the alloy to a temperature slightly below the melting point of the aluminum-beryllium eutectic to cause substantial 115 solution of the undissolved beryllium constituent of the alloy, and thereafter quenching the alloy from substantially said temperature.

2. The method of treating an aluminum base alloy containing not less than about .025% beryllium, which comprises heating the alloy to a temperature slightly below the melting point of the most fusible constituent of the alloy to cause substantial solution of the undissolved beryllium constituent of the alloy, and thereafter quenching the alloy from substantially said temperature.

3. The method of treating an aluminum base alloy containing from about .025 to 130

1.00% beryllium, which comprises heating the alloy to a temperature slightly below the melting point of the most fusible constituent of the alloy to cause substantial solution of the undissolved beryllium constituent of the alloy, and thereafter quenching the alloy from substantially said temperature.

4. The method of treating an aluminum base alloy containing from about .025 to 10 25.0% beryllium, which comprises heating the alloy to a temperature slightly below the melting point of the most fusible constituent of the alloy to cause substantial solution of the undissolved beryllium constituent of the 15 alloy, and thereafter quenching the alloy from substantially said temperature.

5. The method of treating an aluminum base alloy containing beryllium, which comprises heating the alloy to a temperature 20 slightly below the melting point of the aluminum-beryllium eutectic to cause substantial solution of the undissolved beryllium constituent of the alloy, thereafter quenching the alloy from substantially said temperature, 25 and subsequently aging the alloy at a temperature not higher than about 200° C.

6. The method of treating an aluminum base alloy containing not less than about .025% beryllium, which comprises heating 30 the alloy to a temperature slightly below the melting point of the most fusible constituent of the alloy to cause substantial solution of the undissolved beryllium constituent of the alloy, thereafter quenching the alloy from 35 substantially said temperature, and subsequently aging the alloy at a temperature not higher than about 200° C.

7. The method of treating an aluminum base alloy containing from about .025 to 40 1.00% beryllium, which comprises heating the alloy to a temperature slightly below the melting point of the most fusible constituent of the alloy to cause substantial solution of the undissolved beryllium constituent of the 45 alloy, thereafter quenching the alloy from substantially said temperature, and subse-

quently aging the alloy at a temperature not higher than about 200° C.

8. The method of treating an aluminum base alloy containing from about .025 to 50 25.0% beryllium, which comprises heating the alloy to a temperature slightly below the melting point of the most fusible constituent of the alloy to cause substantial solution of the undissolved beryllium constituent of the 55 alloy, thereafter quenching the alloy from substantially said temperature, and subsequently aging the alloy at a temperature not higher than about 200° C.

9. The method of treating an aluminum base alloy containing not less than about .025% beryllium and also containing copper, which comprises heating the alloy to a temperature slightly below the melting point of the most fusible constituent of the alloy to 60 65 cause substantial solution of the undissolved beryllium constituent of the alloy, and thereafter quenching the alloy from substantially said temperature.

10. The method of treating an aluminum base alloy containing not less than about .025% beryllium and also containing silicon and copper, which comprises heating the alloy to a temperature slightly below the melting point of the most fusible constituent 70 75 of the alloy to cause substantial solution of the undissolved beryllium constituent of the alloy, and thereafter quenching the alloy from substantially said temperature.

11. The method of increasing the hardness 80 and tensile strength of an aluminum base alloy containing not less than .025% beryllium, which comprises heating the alloy to a temperature below the melting point of its most fusible constituent, and thereafter 85 quenching the alloy from substantially said temperature.

In testimony whereof, we hereunto sign our names.

ROBERT S. ARCHER.  
WILLIAM L. FINK.